

Patented July 17, 1934

1,966,579

# UNITED STATES PATENT OFFICE

1,966,579

## METHOD OF PREPARING CELLULOSE ACETATES

Van L. Johnson, Waynesboro, Va., assignor to  
Du Pont Rayon Company, New York, N. Y., a  
corporation of Delaware

No Drawing. Application November 10, 1932,  
Serial No. 642,026

4 Claims. (Cl. 260—101)

This invention relates to the production of artificial thread formed of a plurality of cellulose acetates which, upon subsequent treatment with hot water or hot soap solutions, such as at or near the boiling point thereof, or steam, loses a considerable portion of its luster and assumes a dull or mat appearance. More particularly, the instant invention relates to a process of preparing a mixture of cellulose acetates to be used in the production of artificial thread of the type immediately aforementioned.

The Johnson and Swezey application, Serial No. 624,897, filed July 26, 1932, discloses spinning a solution containing a plurality of cellulose acetates having different characteristics, such as different acetyl values (calculated as acetic acid) for the purpose of producing a thread which, upon treatment with steam or hot liquids, such as water or soap solutions at or near the boiling point thereof, will be readily delustered. According to the Johnson and Swezey application, the desired results may be secured if the thread is formed of a plurality of cellulose acetates, such as 50%—95% by weight of a cellulose acetate having an acetyl value, calculated as acetic acid, of 54%—56%, and 5%—50% by weight of a cellulose acetate having an acetyl value, calculated as acetic acid, of 43%—53%. In the preferred embodiment, Johnson and Swezey 30 contemplate a thread composed of 90%—96% of a cellulose acetate having an acetyl value, calculated as acetic acid, of 54%—55%, and 4%—10% of a cellulose acetate having an acetyl value, calculated as acetic acid, of 45%—47%.

I have found that I can produce a thread having the characteristics previously mentioned by spinning, and preferably by the dry spinning process, a solution containing a mixture of acetates having the desired average acetyl value by hydrolyzing a solution containing a plurality of acetates having different acetyl values until the desired average acetyl value of the mixture is secured.

It is, therefore, an object of this invention to provide a method of preparing a mixture of a plurality of cellulose acetates, each of said acetates having different characteristics, which comprises hydrolyzing a solution containing a plurality of acetates having different acetyl values until the desired average acetyl value of the mixture is obtained.

A specific object of this invention is to provide a method of preparing a mixture of a plurality of cellulose acetates which comprises in-

corporating in a solution containing a primary acetate, for example the solution secured at the end of the usual acetylation of cellulose with acetic acid, acetic anhydride and a catalyst, a cellulose acetate having an acetyl value, calculated as acetic acid, different from that of the primary acetate and such as a cellulose acetate having an acetyl value, calculated as acetic acid, of 54%—55%, and then hydrolyzing the mixture of said acetates until the average acetyl value, calculated as acetic acid, of the mixture of the acetates is approximately 53%—54%.

Other objects will appear from the following description and appended claims.

In accordance with the principles of the instant invention, cellulose is acetylated in the usual manner with for example acetic acid, acetic anhydride and a catalyst, such as sulphuric acid, until the primary acetate is produced. At the end of the acetylation operation, the primary cellulose acetate is dissolved in the acetic acid, and to this solution there is added a predetermined quantity of a cellulose acetate which is characterized by an acetyl value different from that of the primary acetate. After thoroughly mixing, the mixture is hydrolyzed as is well known in the art until the desired average acetyl content of the mixture of the acetates is secured. The resulting mixed acetate in the mass are then precipitated with water, washed, and dried in the usual manner.

The product of the foregoing procedure is a homogeneous and uniform mixture of acetates and forms, when dissolved in appropriate solvents, a spinning solution which upon being spun, for example by the dry spinning process, produces a thread which upon treatment with steam or hot liquids, such as water or soap solutions, at or near the boiling point thereof, will be readily delustered.

It is obvious that the quantity of cellulose acetate added to the solution containing the primary acetate depends partly upon the relative quantities of the different cellulose acetates desired in the mixture. Likewise, the acetyl value, calculated as acetic acid, of the cellulose acetate added to the solution of the primary acetate depends partly on the average acetyl mixture desired in the final product. Satisfactory results have been secured when 5%—20% of cellulose acetate having an acetyl value, calculated as acetic acid, of approximately 54%—55% was added to the primary acetate solution and the hydrolysis continued until the

average acetyl value, calculated as acetic acid, was approximately 53%-54%.

In the preferred embodiment of the invention, the cellulose acetate which is added to the primary acetate solution is preferably soluble therein. In one embodiment of the invention, the added cellulose acetate may be in the finely divided state. Alternatively, the added acetate may be previously dissolved in a suitable solvent, such as acetic acid, and then added to the primary acetate solution.

In order to explain more fully the principles of this invention, the following illustrative example is set forth. It is, of course, to be understood that the invention is not restricted thereto but is merely illustrative.

*Example.*—To 21.6 parts of cellulose acetate in solution in acetic acid at the end of the primary acetylation there is added 2.4 parts of cellulose acetate having an acetyl value, calculated as acetic acid, of 54%-55%, either in the form of finely ground material or in solution in acetic acid. After thoroughly mixing the same, the mass is subjected to the well-known hydrolysis operation which is continued until the average acetyl values of the mixture of cellulose acetates is approximately 53%-54%. At this time, the resulting mixed acetate is precipitated with water, washed, and dried in the usual manner.

The resulting product is a heterogeneous mixture of the plurality of acetates. A predetermined quantity of this mixture of acetates is then dissolved in appropriate solvents, such as acetone, or acetone and alcohol, to produce a spinning solution of suitable concentration, such as, for example, one containing 20%-30% of said mixture of acetate. Upon spinning such a solution by the dry spinning process there is obtained a thread which is characterized by a normal luster. The thread either prior to or subsequent to weaving or knitting into cloth, when subjected to, for example, a boiling 2% soap solution for approximately 1 hour, acquires or assumes a dull or mat appearance.

Though the invention has been particularly described in connection with a mixture of two acetates of different characteristics, it is to be understood that the invention is not restricted thereto, since it is obvious that more than two acetates may be employed with equal success. Also, the method herein described is equally

applicable to the production of mixed acetates for any purpose.

Since it is obvious that various changes and modifications may be made in the above description without departing from the nature or spirit thereof, this invention is not restricted thereto except as set forth in the appended claims.

I claim:

1. A method of preparing a mixture of a plurality of cellulose acetates, each of said acetates having different characteristics, which comprises acetylating cellulose until a primary cellulose acetate is produced, incorporating in the primary acetate solution a cellulose acetate having an acetyl value different than said primary acetate, and hydrolyzing the acetates until the desired average acetyl value of the mixture of acetates is secured. 85

2. A method of preparing a mixture of a plurality of cellulose acetates, each of said acetates having different characteristics, which comprises acetylating cellulose until a primary acetate is secured, incorporating a cellulose acetate having an acetyl value, calculated as acetic acid, of approximately 54%-55% in the solution containing said primary acetate, and hydrolyzing the acetates until the average acetyl value, calculated as acetic acid, of the mixture of acetates is approximately 53%-54%. 90

3. A method of preparing a mixture of a plurality of cellulose acetates, each of said acetates having different characteristics, which comprises acetylating cellulose until a primary acetate is secured, incorporating 5%-20% of a cellulose acetate having an acetyl value, calculated as acetic acid, of approximately 54%-55% in the solution containing said primary acetate, and hydrolyzing the acetates until the average acetyl value, calculated as acetic acid, of the mixture of acetates is approximately 53%-54%. 105

4. A method of preparing a mixture of a plurality of cellulose acetates, each of said acetates having different characteristics, which comprises acetylating cellulose until a primary acetate is secured, incorporating a cellulose acetate having an acetyl value, calculated as acetic acid, of approximately 54%-55% in the solution containing said primary acetate and in such an amount as to constitute 10% of the combined acetates, and hydrolyzing the acetates until the average acetyl value, calculated as acetic acid, of the mixture of acetates is approximately 53%-54%. 110

VAN L. BOHNSON.

55

130

60

135

65

140

70

145

75

150